# EUROPEAN PATENT APPLICATION

(11) **EP 0 272 652 A2**
(43) Date of publication of application: **29.06.1988**
(21) Application number: 87118859.5
(22) Date of filing: 18.12.1987
(51) Int. Cl.: H01J 61/12, H01J 61/82, H01J 61/18

(54) **Scandium oxide additions to metal halide lamps**

(30) Priority: 18.12.1986 US 943981
(71) Applicant: GTE PRODUCTS CORPORATION, Wilmington Delaware 19801 (US)
(72) Inventor: Duggan, George K., Bedford, Massachusetts 01966 (US); Keeffe, William M., Rockport, Massachusetts 01966 (US)
(74) Representative: Grünecker, Kinkeldey, Stockmair & Schwanhäusser Anwaltssozietät

(57) **Abstract**

In its most preferred embodiments, the present invention thus represents an improved Na-Sc-I lamp, wherein the improvement consists essentially of the addition of at least about 1 mg of particulate polycrystalline scandia to the arc tube.

The positive benefits derived from this incorporation of PCS include improved lamp performance over long periods of time (e.g., 8000 hrs.) including improved lumen output, and improved maintenance and retention of CRI.

## Description

### FIELD OF THE INVENTION

The present invention relates to improvements in metal halide lamps, and particularly to metal halide lamps containing scandium as a light radiating additive.

### BACKGROUND OF THE INVENTION

Metal halide lamps combine the high luminous efficacy and good color rendition of fluorescent lamps with the high power compact-source characteristics of high pressure mercury lamps. As a result, these lamps overcome many of the deficiencies of both earlier lamp types, and are capable of better serving many of the applications that had previously been the mainstays of the earlier lamp types.

Metal halide lamps generally consist of a quartz arc tube with two main electrodes, jacketed in a hard glass envelope. The arc tube itself contains a rare gas (e.g., argon) for starting and a charge of mercury, plus one or more of the metal halides (usually iodides). For a description of typical metal halide lamp construction, see U.S. Patent No. 3,424,935 to Gungle et al.

During the operation of a metal halide lamp, all of the mercury is vaporized, resulting in a high-pressure, wall-stabilized arc in a gas consisting principally of mercury vapor at several atmospheres pressure. The metal iodides are also vaporized and ultimately dissociated. The metal atoms are excited and ionized in the high temperature arc column, and they give off their characteristic spectral lines. As the metal atoms diffuse back to the walls of the arc tube, they encounter iodine atoms and recombine to form iodide molecules.

One of the problems typically encountered in scandium (Sc) containing metal halide lamps is the steady decrease of both lumen maintenance and color rendering index (CRI) over the life of the lamp. This is believed to be due to reactions between one or more of the fill components, e.g., HgI₂, NaI, Hg and Sc, and the quartz arc tube or the tungsten electrodes.

One result of these chemical interactions is the steady reduction in the amount of scandium. For example, scandium, present in the arc tube as ScI₃, can react with the quartz wall of the arc tube according to the following equation:

4 ScI₃ (g) + 7 SiO₂ (s) → 2 Sc₂Si₂O₇ (s) + 3 SiI₄

The progressive loss of Sc over the life of the lamp effects not only lumen maintenance and CRI, but also results in an increase in free iodine, which causes the lamp voltage to rise, and may ultimately cause lamp failure.

One prior art response to the progressive loss of scandium which occurs in these metal halide lamps was the addition of a small chip or disc of scandium metal to the fill of the lamp. The theory behind such an additional component being that excess Sc would thus be available for the reactions that would otherwise deplete the necessary fill component.

Unfortunately, under the operating conditions of typical metal halide lamps, this is not the case. In fact, excess scandium reacts with the quartz arc tube at lamp operating temperatures, according to the following empirical relation:

Sc (s) + SiO₂ (s) → Sc₂Si₂O₇

While this Sc₂Si₂O₇ can further react with SiI₄ to form ScI₃ according to the following equation:

3 SiI₄ (g) + 2 Sc₂Si₂O₇ (s) → 4 ScI₃ (g) + 7 SiO₂

such a reaction must await the formation of the proper components.

Another attempt at solving the scandium consumption problem was proposed by Inoue in Japanese Patent Application No. 55-165324. This case employed the addition of an alumina ceramic body containing both Sc₂O₃ and Sc. In theory, excess I₂ generated during lamp life would diffuse into the alumina ceramic body, to react with, and to bring the free Sc into the arc.

Several attempts have been made to incorporate scandium into other portions of metal halide lamps i.e., other than as fill components. For example, U.S. Patent No. 4,594,220 to Rigden, describes the use of scandium oxide in the electrodes of metal halide lamps, stating that, "it is essential that the scandium oxide is incorporated into the electrode structure by melting" (see, column 2, lines 21-23) and that the "scandium oxide (is an) activator" (see, column 2, line 67).

In Japanese Patent Application No. 58-129741 to Ishigami et al., the use of scandium oxide as part of the electrode coil in metal halide lamps is described (see, e.g., p.1, line 6; p. 4, lines 7 and 8; p. 5, line 27; p.6, line 1; and p.8, line 3).

Similarly, in Japanese Patent Application No. 57-74959 to Saito et al., the use of scandium oxide in metal halide lamps is suggested as "(an) electrode having an electron radiation substance containing scandium oxide" (p.1, lines 4, and 5).

Although scandia has been previously employed in metal halide lamps, another reason to avoid adding scandia to the fill of a metal halide lamp is the possibility of a chemical reaction occurring between the Sc₂O₃ and the electrode (W), which is known to occur at temperatures in excess of 2100°C (the filament temperature will be at least this high). See for example, Horovitz et al., Scandium, Academic Press, New York, (1975).

In spite of the apparent drawbacks described in the prior art, the present inventors added particulate polycrystalline scandia to the fill of metal halide lamps, resulting in the surprising benefits described herein below.

### SUMMARY OF THE INVENTION

The present invention is directed to a metal halide discharge lamp comprising: an arc tube having spaced electrodes, and containing a fill including a starting gas, mercury, and metal halides; the fill further including a fill component consisting essentially of an effective amount of particulate polycrystalline scandia, said polycrystalline scandia containing from about 0 to 0.5 weight percent alumina; and an outer envelope enclosing said arc tube.

In its most preferred embodiments, the present invention thus represents an improved Na-Sc-I metal halide lamp, wherein the improvement consists essentially of the addition of at least about 1 mg of particulate polycrystalline scandia to the arc tube.

The positive benefits derived from this incorporation of PCS include improved lamp performance over long periods of time (e.g., 8000 hrs.) including improved lumen output, and improved lumen maintenance and retention of CRI.

### BRIEF DESCRIPTION OF THE FIGURES

Figure 1 shows the effect of Sc₂O₃ addition of the lumen output of 400W Metalarc● lamps during life.
Figure 2 illustrates the variation in the intensity of the 508 nm Sc line with Sc₃O₃ weight and life.
Figure 3 illustrates the variation in the intensity of the 610 nm Na line with Sc₂O₃ weight and life.
Figure 4 illustrates the ratio of (Na/Sc)condensed for the three test groups.
Figure 5 illustrates the effect of Sc₂O₃ addition on the average lamp voltage at 400W during life test.
Figures 6-8 are chromaticity diagrams illustrating the effect of various amounts of added polycrystalline scandia to the normal fill of 400W Metalarc● lamps:
Figure 6 is the plot of a test group of lamps, each containing less than about 10 mg of PCS fill additive;
Figure 7 is the plot of a test group of lamps, each containing greater than about 10 mg of PCS fill additive; and
Figure 8 is the plot of the control group of lamps, each with no added PCS.

### DETAILED DESCRIPTION OF THE PREFERRED EMBODIMENTS

The preferred metal halide lamp improved by means the present invention is the Sylvania Metalarc● lamp.

Sylvania's Metalarc● lamp is a member of the high intensity discharge (H.I.D.) lamp family and provides an efficient source of white light. It has high efficacy, long life, good color rendering ability and lumen maintenance.

Physically, Metalarc● lamps are compact in size and have approximately the same outside dimensions as corresponding wattage mercury lamps. Metalarc● lamps are available in broad range of sizes in wattages from 100 to 1,500, lumen packages from 8,500 to 155,000 and in a range of color temperatures, from 3200K (warm white light) to 4500K (white light).

Such lamps are widely used in the USA, but they differ from European metal halide lamps in arc tube construction, additive chemistry and type of ballasting employed.

The Metalarc● lamp has a quartz arc tube which is slightly smaller than that of the same wattage mercury lamp. The arc tube contains argon gas as a starting gas, as well as mercury, sodium and scandium iodides as radiative additives. The iodides are responsible for the outstanding performance of this light source. The ends of the arc tube have a heat reflecting coating to control the temperature of these areas during operation.

The Metalarc● lamp uses a split frame construction. This is necessitated by the high photoelectrical activity of the additives which requires maximum possible isolation of metal parts from the arc tube.

The arc tube harness includes spring supports at the neck and dome, which make the mount structure very durable and resistant to shocks and vibration. The bimetal shorting switch in the Metalarc● lamp closes during lamp operation, providing a short circuit between the starting electrode and the adjacent main electrode. This prevents voltage drop between the main electrode and the starting electrode which can lead to electrolytic failure of the arc tube seal.

Some Metalarc● lamps use a solid state diode and a bimetal switch. The diode augments the bimetal switch during lamp warmup. A borosilicate (hard) glass outer jacket protects the inner parts and also absorbs ultraviolet light from the arc.

While not wishing to be bound by theory, the following represents one possible mechanism to explain the benefit in lamp performance discovered by the addition of polycrystalline scandia (Sc₂O₃) to Metalarc● lamps as a fill component.

Scandium present as ScI₃ in Metalarc● lamps may be lost through reaction with the quartz wall as:

1. 4 ScI₃(g) + 7 SiO₂(s) → 2 Sc₂Si₂O₇(s) + 3 SiI₄

or with water vapor as:

2. 2 ScI₃(s) + 3 H₂O(s) → Sc₂O₃(s) + 6 HI(g).

In Reaction 1, the formation of SiI₄ also causes melt back at the electrode via the empirical reaction,

3. SiI₄(g) + W(g) ↔ WSi₂(s)

while in Reaction 2, the HI will react with Hg to form HgI₂. This will thermally dissociate yielding excess iodine which reduces lamp performance, leads to increased arc tube blackening rate, and increases reignition voltage.

To overcome the loss of ScI₃ with time and the formation of excess I₂ or iodine compounds, the prior art would add a Sc chip as part of the fill to the arc tube. The Sc chip, however, reacts rapidly with the quartz wall at lamp operating temperatures as:

4. Sc(s) + SiO₂(s) → Sc₂Si₂O₇.

But Sc₂Si₂O₇ may then react with SiI₄ to form ScI₃ via:

5. 3 SiI₄(g) + 2 Sc₂Si₂O₇(s) → 4 ScI₃(g) + 7 SiO₂(s).

The present invention allows for the direct reaction of SiI₄ with the Sc₂O₃ additive via:

6. 7 Sc₂O₃(s) + 6 SiI₄(g) → 8 ScI₃(g) + 3 Sc₂Si₂O₇.

The Sc₂Si₂O₇ reaction product of Reaction 6 thus provides additional reactant for Reaction 5, thereby providing an additional chemical pathway for the removal of the undesirable SiI₄ and the synthesis of the desired ScI₃.

This dual cyclic path leads to more efficiently sustaining the vapor phase Sc through the volatile ScI₃ specie, as shown in the life test results described below, with resulting better lumen output.

Lamp tests were conducted using three lamp groups;
(A) The first group, the "<10 mg group," had Sc₂O₃ additions of 0.004, 0.004, 0.007 and 0.012 g.
(B) The second group, the ">10 mg group," had Sc₂O₃ additions of 0.021, 0.024, 0.027, 0.028, 0.074 and 0.136 g.
(C) The third group, the "control group," had no Sc₂O₃ added to the typical fill of a 400W Metalarc● lamp (in this case, 20.7 mg NaI, 3.8 mg HgI₂, 49 mg Hg, and 0.5 mg Sc).

Figure 1 shows the effect of Sc₂O₃ weight on lumen output versus time. After 5000 hours life, test lamps were 13.5 and 8.5% higher in lumen output for the <10 mg Sc₂O₃ and >10 mg Sc₂O₃ groups, respectively, versus the control lamps (four lamps). T-test analysis of the data indicates a 97.5% confidence level that there is a significant difference between the average value for the control lamps and the scandia containing lamps.

The improved lumen output may be attributed to higher retention of Sc in the arc (Figure 2). The 508 nm Sc spectral line, while optically thin, shows a higher Sc intensity for both test groups as compared with the control lamps. This compares favorably with the very slight drop in the intensity of the 610 nm Na line for the two test groups versus the control group (Figure 3).

The retention of Sc can also be seen from the results in Figure 4. Here, the average ratio of (Na/Sc)condensed is shown for the lamp groups over the life of the test. The ratio (Na/Sc)condensed is calculated from Raoult's Law and based on the vapor pressures of Na and Sc in a burning lamp as detected by a polychromator.

As shown in Figure 4, the (Na/Sc)condensed for the Sc₂O₃ containing groups is constantly lower than that of the control and significantly so, as shown in Figure 2, for the "Sc₂O₃ >10 mg group." This indicates the higher retention of Sc with Sc₂O₃ addition or a continued supply of Sc during the course of the lamp life.

A further benefit of the Sc₂O₃ addition is lower lamp voltage in the test groups. The average lamp voltage at 400W stayed fairly close (Figure 5) over the first 2000 hours of life but then began to diverge. At 5000 hours, the controls showed the highest lamp voltage (137.9 volts) being 2.4 volts higher than the "<10 mg Sc₂O₃ group" and 3.0 volts higher than ">10 mg Sc₂O₃ test group."

The test of the addition of various amounts of polycrystalline scandia (PCS) to the fill of otherwise standard 400 Watt Metalarc● lamps has reached 8,000 operating hours under standard life test conditions (10 hours on /2 hours off).

The results are shown in the attached chromaticity plots, which show the color coordinate data points of the individual lamps in each of the three test groups.

Figure 6 shows the data for the "< 10 mg group" of PCS additive, while Figure 7 shows the data for the "> 10 mg group" of PCS additive. Figure 8 is the control group without added PCS.

The mean value of the y-coordinate is an effective measure of the scandium radiation which is dependent upon the scandium concentration within the arc tube. The control group in Figure 8 shows a mean y-value of 0.347 which is well below the design center y-value of 0.385 and evidential of the scandium loss problem characteristic of long term ageing of standard Metalarc● lamps.

The mean y-value of the small addition ( i.e., the "< 10 mg group") in Figure 6, shows a higher value of 0.364 evidential of scandium replenishment by the PCS thereby offsetting some of the loss seen in the control group. Moreover, the group having the heavier additions (i.e., the "> 10 mg group") in Figure 7, shows even greater enhancement (y = 0.369), confirming that the amount of scandium replenishment is proportional to the quantity of PCS added.

The present invention will be further illustrated with reference to the following examples which aid in the understanding of the present invention, but which are not to be construed as limitations thereof. All percentages reported herein, unless otherwise specified, are percent by weight. All temperatures are expressed in degrees Celsius.

### EXAMPLE

The Sc₂O₃ powder was transformed into a polycrystalline ceramic body at GTE Laboratories Incorporated, Waltham, Massachusetts before being added to the arc tube.

In this process, Sc₂O₃ powder plus a small Al₂O₃ addition (up to 0.5 w/o) was pressed into a disc and then subjected to solid state sintering according to the following sintering schedule:

The resultant polycrystalline scandia was cut into small, thin slices and weighed. The 400W Metalarc● lamps were then prepared by adding various weights of Sc₂O₃ ranging from 4 to 136 mg to the arc tubes along with 57 mg Hg, 3.8 mg HgI₂, 20.7 mg NaI, 0.5 mg Sc and 32 Torr of Ar.

The lamps were aged horizontally and removed at specific times in order to determine the electrical and SPD parameters.

From the test results reported above, it was determined that the minimum effective amount of PCS necessary to improve a 400W Metalarc● lamp was about 1 mg. Using this as a minimum PCS value, and knowing the volume of the 400W Metalarc● lamp arc tube (i.e., 13.8 cc), the effective amount of PCS necessary to improve any other metal halide lamp may be expressed as a given weight per arc tube volume, i.e., about, 0.072 mg/cc.

Thus, to extend this invention to any other scandium containing metal halide lamp, the minimum amount of PCS that would be expected to show any beneficial effect would be at least about 0.07 mg per cc of arc tube volume.

The present invention has been described in detail, including the preferred embodiments thereof. However, it will be appreciated that those skilled in the art, upon consideration of the present disclosure, may make modifications and/or improvements on this invention and still be within the scope and spirit of this invention as set forth in the following claims.

## Claims

1. A metal halide discharge lamp comprising:
an arc tube having spaced electrodes, and containing a fill including a starting gas, mercury, and metal halides;
the fill further including a fill component consisting essentially of an effective amount of particulate polycrystalline scandia, said polycrystalline scandia containing from about 0 to 0.5 weight percent alumina; and
an outer envelope enclosing said arc tube.

2. The metal halide lamp of claim 1, wherein the fill includes NaI, HgI₂, Hg, and Sc.

3. A method of improving the lamp maintenance and color rendering index of metal halide lamps having sodium and scandium as fill components, said method consisting of adding an effective amount of particulate poIycrystalline scandia to the fill.

4. The method of claim 3, wherein the metal halide lamp has fill components consisting of NaI, HgI₂, Hg, and Sc.

5. The method of claim 4, wherein the effective amount of particulate polycrystalline scandia is at least about 1 mg.

6. The method of claim 5, wherein the effective amount of particulate polycrystalline scandia is less than about 10 mg.

7. The method of claim 5, wherein the effective amount of particulate polycrystalline scandia is greater than about 10 mg.

8. A method of forming polycrystalline scandia suitable for use as a fill component in a metal halide lamp, said method comprising pressing scandium oxide powder into a compact mass and subjecting the compact mass to solid state sintering at an elevated temperature, under a first atmosphere consisting essentially of dry hydrogen, then under a second atmosphere consisting essentially of wet hydrogen, for a sufficient time to produce polycrystalline scandia.

9. The method of claim 8, wherein the scandium oxide powder further includes up to about 0.5 percent by weight alumina.

10. The method of claim 8, wherein the solid state sintering temperature is up to about 2000°C.
